

UNITED STATES PATENT OFFICE

2,283,573

METHOD OF ~~WATERPROOFING~~ AND PREVENTING EFFLORESCENCE OF MORTAR IN MASONRY

James B. Pierce, Jr., Charleston, W. Va., assignor to Standard Ultramarine Company, Huntington, W. Va., a corporation of West Virginia

No Drawing. Application December 24, 1938,  
Serial No. 247,645

5 Claims. (Cl. 106—314)

This invention relates to the prevention of efflorescence of mortar in brick, tile and like masonry walls and has for its principal objects the provision of an efficient and economical method of preventing such efflorescence besides effecting the substantial if not complete waterproofing of such mortar. Other objects of the invention are hereinafter set forth.

Heretofore, as I am well aware, the stearates of either calcium, aluminum and ammonium have been employed for the purpose of rendering masonry walls waterproof. While these products are highly water-repellent and therefore adapted for retarding the penetration of moisture through a masonry wall, whether the same be due to faulty coping, bad flashing or otherwise, nevertheless, they are wholly ineffective for preventing the efflorescence of the mortar employed in laying up brick, tile and other masonry walls since they are incapable of fixing sulphates of alkali and alkaline earth metals, which salts are the prime cause of such efflorescence. Moreover the waterproofing action of stearates of calcium, aluminum and ammonium, however, is not by any means perfect and even when considerable quantities of these stearates are added to the mortar, for example up to 3%, some moisture will pass through the mortar, after the same is set, especially after severe weather conditions and when this occurs efflorescence in the wall is bound to appear.

My investigations have led to the discovery that barium stearates possess all the desirable waterproofing qualities of the aforesaid stearates and in addition thereto, reacts with the sulphates of alkali and alkaline earth metals to form insoluble barium sulphate and the corresponding alkali or alkaline earth stearates, thereby functioning as an effective efflorescence preventative, besides serving as an effective waterproofing compound, when incorporated with the mortar of such wall prior to the laying up of the wall. Furthermore, although the barium stearate may not be, under the most severe conditions, an absolute waterproofing agent for masonry, nevertheless whatever moisture passes through a wall, which has been subjected to the herein-after described treatment with barium stearate, will not act as a carrier or vehicle for soluble efflorescence-producing sulphates, such as aforesaid, due to the fact that such sulphates react with the waterproofing and efflorescence-prevention agent and, as a consequence, insoluble barium sulphate and the corresponding alkali and alkaline earth stearates will be formed in

situ in the mortar of such brick, tile or like masonry walls while the moisture will collect on the surface of the wall as an innocuous film which evaporates without leaving a trace of efflorescence.

As an example of the preferred manner of waterproofing and preventing efflorescence of mortar in brick, tile and other masonry walls laid up with mortar, the following is submitted: Equi-molecular proportions of solid stearic acid is added, with constant stirring, to concentrated barium sulphide liquor of from 10% to 20% BaS content whereupon the same react to form insoluble barium stearate in the form of a flocculent precipitate and hydrogen sulphide gas (H<sub>2</sub>S). The precipitate is thoroughly washed with water to free the same from occluded H<sub>2</sub>S, then filtered, dried and powdered in accordance with standard processing methods.

In the treatment of mortar intended for use in the laying up of masonry walls of the aforesaid types, an amount of barium stearate, produced as aforesaid, equal to  $\frac{1}{2}\%$  to 3% by weight of the amount of mortar, whether lime mortar or Portland or other cement mortar be employed in laying up the wall, is intimately admixed with the mortar, while the latter is in the usual sloppy state and such mortar while still fresh is then employed to lay up the desired brick, tile or like masonry wall. But about  $\frac{1}{2}\%$  of barium stearate is usually effective in preventing subsequent efflorescence in the wall so laid up with the mortar treated as aforesaid but an amount of 3% of such stearate will insure absolute protection against any such efflorescence even under the most severe conditions. However, except in those cases where the coping and/or flashing is poor and very severe weather conditions are experienced accompanied by alternate freezing and thawing over several months at a time, the smaller amount of barium stearate, namely but about  $\frac{1}{2}\%$ , usually suffices to afford very satisfactory protection. In addition to serving as an effective efflorescence preventative in an outside wall, such barium stearate can also be advantageously employed as an ingredient in the mortar of the back-up tile or other similar lining material of a wall, since whatever moisture may enter the masonry wall will pass into the mortar of the back-up tile and, when the wall again dries, since the outer wall dries first, it will pull the moisture outwardly into itself whence it passes outwardly and evaporates, thus effectively protecting the back-up tile against being discolored or disfigured by ugly efflorescence stains.

The wet or sloppy mortar mix herein referred to is that commonly prepared from slaked lime, either water or air-slaked lime or from Portland or like cement in admixture with the requisite amount of water and sand, crushed marble or other inert granular material commonly employed to form a mortar of the usual consistency and lime or cement content. As is well known in the case of ordinary lime mortar, the calcium hydrate is essentially converted on aging to calcium carbonate.

While my method of prevention of efflorescence has been particularly described with reference to the treatment of the lime or cement mortar of masonry walls laid up with such mortar, it is also equally applicable for the prevention of efflorescence in any form of unburnt, fabricated building blocks or slabs, as for example Portland cement blocks, unburnt brick or unburnt artificial tile, since such barium stearate is equally effective in preventing efflorescence in such blocks or slabs, as well as mortar, provided it is not heated to a temperature in excess of its decomposition point.

While I have specified certain preferred proportions of ingredients in the production of the barium stearate and in carrying out the aforesaid treatment for preventing efflorescence in masonry walls, various changes in such proportions and in the exact method of procedure, herein outlined, may be made without departing from the spirit of my invention as embraced within the scope of the appended claims.

Having thus described my invention, what I claim and desire to obtain by United States Letters Patent is:

1. The method of making a highly water-repellent and substantially non-efflorescent mortar for masonry, comprising incorporating with a mortar, belonging to the group consisting of lime mortar and Portland cement mortar and containing an appreciable amount of a water-soluble, efflorescence-forming compound belonging to the group consisting of an alkali metal sulphate and an alkaline earth metal sulphate, an amount of barium stearate which is at least substantially the chemical equivalent of any such water-soluble compound and effecting thereby the precipitation in situ in such mortar of barium sulphate and calcium stearate.

2. The method of making a highly water-repellent and substantially non-efflorescent mortar for masonry, comprising incorporating with a mortar, belonging to the group consisting of lime mortar and Portland cement mortar and

containing an appreciable amount of a water-soluble, efflorescence-forming compound belonging to the group consisting of an alkali metal sulphate and an alkaline earth metal sulphate, 5 an amount of barium stearate which is from  $\frac{1}{4}\%$  to 5% of the weight of the solid content of the mortar and which is at least substantially the chemical equivalent of any such water-soluble compound and effecting thereby the precipitation in situ in such mortar of barium sulphate and calcium stearate.

3. A waterproof and substantially non-efflorescent mortar belonging to the group consisting of lime mortar and Portland cement mortar and 15 containing barium sulphate and calcium stearate each precipitated in situ therein, the amount of the stearate radical in such precipitated calcium stearate being the chemical equivalent of an amount of barium stearate equal to from  $\frac{1}{4}\%$  to 5% by weight of the solid content of the mortar but not substantially exceeding the chemical equivalent of the barium radical in such precipitated barium sulphate and substantially the sole waterproofing agent present in said mortar comprising a stearate of an alkaline earth metal.

4. A waterproof and substantially non-efflorescent mortar belonging to the group consisting of lime mortar and Portland cement mortar and containing barium sulphate and calcium stearate each precipitated in situ therein, the amount of the stearate radical in such precipitated calcium stearate being the chemical equivalent of an amount of barium stearate equal to from  $\frac{1}{4}\%$  to 3% by weight of the solid content of the mortar but not substantially exceeding the chemical equivalent of the barium radical in such precipitated barium sulphate and substantially the sole waterproofing agent present in said mortar comprising a stearate of an alkaline earth metal.

5. A waterproof and substantially non-efflorescent mortar belonging to the group consisting of lime mortar and Portland cement mortar and containing barium sulphate and calcium stearate 45 each precipitated in situ therein, the amount of the stearate radical in such precipitated calcium stearate being the chemical equivalent of an amount of barium stearate equal to about  $\frac{1}{2}\%$  by weight of the solid content of the mortar but not substantially exceeding the chemical equivalent of the barium radical in such precipitated barium sulphate and substantially the sole waterproofing agent present in said mortar comprising a stearate of an alkaline earth metal.

JAMES B. PIERCE, JR.